

**1**

3,353,989

**METHOD OF PRODUCING N-CHLORAMIDE VESICANT PROTECTIVE FABRIC AND THE RESULTING FABRIC**

Carlo G. De Marco, Cochituate, Mass., assignor to The United States of America as represented by the Secretary of the Army  
No Drawing. Filed June 16, 1964, Ser. No. 375,673  
5 Claims. (Cl. 117—62.1)

**ABSTRACT OF THE DISCLOSURE**

A permanent vesicant protective, resin finish for fabric materials formed by curing methylol derivatives of nitrogenous resin-forming materials in situ, said resin having sites which will react with halogen ions to form N-chloramides.

The invention described herein, if patented, may be manufactured and used by or for the Government for governmental purposes without the payment to me of any royalty thereon.

This invention relates to a vesicant resistant finish for fabrics and more particularly, a permanent resin finish for porous fabrics which can be readily and easily converted to a vesicant vapor-resistant finish.

Personnel exposed to vesicant agents, in addition to respiratory protection, require some form of protective covering to shield the body from attack by these agents. While an impermeable garment would afford complete protection by virtue of its ability to exclude all vapors or gases, such garments are not suitable for use for other than extremely brief periods of time because of discomfort to the wearer resulting from the accumulation of water vapor within the garment. A permeable garment having built-in vesicant protection would be preferred both for reasons of comfort and because it would eliminate the need for a special purpose garment.

It is known that vesicant agents, e.g., mustard and organic chloroarsines, are inactivated by reaction with halogens. Various compounds containing halogens in a form suitable for reaction with vesicant agents have been applied to porous fabrics to create a barrier to vesicant vapors. Such compounds have been applied as dusts or in a liquid vehicle to the fabric and are loosely deposited on the surface of the fabric fibers. Attempts to increase the retention of the protective materials on the fabrics by use of binders have not been satisfactory because such materials are usually tacky in nature, have poor resistance to laundering and, in some instances, have an adverse effect on the strength of the fabric. Additionally, clothing containing anti-vesicant halogen materials cannot be hot pressed without serious loss of fabric strength, as the high temperatures involved tend to break down the halogen containing compounds and releasing hydrochloric acid which severely attacks and degrades the cellulosic fibers.

It is among the objects of the present invention to provide a treatment for air-permeable fabric materials having at least a 50% cellulosic content that will prevent the passage of vapors of vesicant agents through the fabric. It is a further object to provide a permanent, non-injurious resin finish for such fabric materials which can be simply and readily reacted with a halogenating agent to form a vesicant-resistant finish and which can be further treated to remove the halogen agent from the resin finish. It is a further object to provide a vesicant-resistant treatment for textile fabrics that is relatively stable, can easily be brought up to full strength, and does not adversely affect the tensile strength of the fabric.

**2**

The objects of my invention are accomplished by treating permeable fabrics, having at least a 50% cellulosic content by weight, with certain nitrogenous resin-forming materials which are cured on the fabric to form an insoluble and permanently fixed resin finish. This resin-treated fabric is capable of reacting with halogen ions, e.g., chlorine ions, and holding the halogen in a labile state, capable of reacting with and inactivating the vapors of mustard or organic chloroarsines. When the presence of the halogen is no longer required or desired, it may be removed from the resin by rinsing the fabric in a water solution containing a reducing agent.

Textile fabrics which are suitable for treatment according to my invention include fabrics composed of hydrophilic, fibrous, cellulosic materials such as cotton and rayon, and also blends of such materials and non-cellulosic synthetic fibers containing at least 50% by weight of the cellulosic material, e.g., 50/50 intimate blends of nylon and cotton, 40/60 blends of polyethylene terephthalate and cotton. While fabrics woven of these fibers will be permeable to the passage of gases and vapors, it is preferred that the permeability to air not exceed 20 cu. ft./minute/sq. ft. at  $\frac{1}{2}$  inch of water pressure.

The nitrogenous resin-forming materials which are operable in my invention include all of those which will form resins having sites which will react with halogen ions to form N-chloramides. Included among these are the methylol derivatives of dicyandiamide, urea, alkyl-substituted urea and melamine, e.g., mono-, di- and trimethyloldicyandiamide, mono-, di- and trimethylol ethyleneurea, mono-, di- and trimethylolurea, methylolmelamine, etc.

The materials are incorporated in a liquid vehicle such as aqueous solutions, suspensions, acid colloids or emulsions in amounts varying from about 5% to about 25% by weight. A condensation catalyst is normally included in the solution which serves to speed up the curing process. Catalysts may be of the acid or alkaline type such as carbonates, organic amines or acid-forming catalysts, e.g., sodium bicarbonate, glycollic acid, alkanolamine salts, and magnesium chloride.

The fabric is treated by dipping into a solution of the resin-forming material followed by mechanical removal of excess liquid to effect a wet pickup of from 40 to about 45% by wt. The impregnated material is then dried at temperatures below 250° F. The dried fabric is cured at an elevated temperature of from about 250° to about 350° F. for a brief period of time, usually from about 3 to less than 10 minutes. Alternatively, the resin may be subjected to a wet steam cure, i.e., curing in the presence of steam at a temperature of approximately 210° F. for 45 to about 120 minutes. Following the curing step the fabric is washed to remove catalyst and any unreacted materials. It is preferred that the resin add-on should be from 10% to about 15% based on the dry weight of the fabric as this amount will not produce objectionable stiffening, loss of strength, or reduction of permeability of the fabric and will provide, when halogenated, excellent resistance to vesicant penetration. The cured resin is insoluble and permanently fixed to the fabric.

Halogenation of the resin is accomplished by immersion of the resin finished fabric in an aqueous solution containing positive halogen ions. Examples of suitable sources of halogen ions include sodium, calcium and lithium hypochlorites and sodium dichloroisocyanurate. It is preferred that there be effected a chlorine concentration of 0.1 to 1.0 mg. of elemental chlorine per sq. cm. of fabric.

**Example I**

70 A resin-forming impregnating solution is prepared by slowly adding 750 grams of monomethyloldicyandiamide to a water-acid mixture of 250 grams of 85% phosphoric

acid and 337 grams of water (70° F.). The mixture is heated to 100° F. at which temperature the reaction becomes exothermic and ice is added (250 grams) to keep the temperature below 110° F. The material is completely dissolved in approximately 30 minutes whereupon the solution is diluted with 915 grams of water at 70° F.

The solution is applied to cotton sateen cloth (9.0 oz.) by means of 2 dips and 2 nips. After application, the fabric is dried at a temperature of 250° F. and cured at 350° F. for 3 minutes. After curing, the treated fabric is rinsed in tap water for about 3 minutes and again dried at 250° F. The treated fabric had a dry add-on of approximately 12% based on the dry weight of the cloth.

The fabric with its permanent resin finish is now in a form whereby whenever it is desired to do so it may be converted to an anti-vesicant finish by reaction with chlorine. The chlorination treatment is quite simple and merely requires that the resin-treated fabric be immersed in a water solution containing positive chlorine ions. The fabric of this example was immersed in a water solution containing 2.5% available chlorine for 15 minutes and then rinsed and dried. The source of chlorine was sodium dichloroisocyanurate. After two days' storage the fabric was analyzed and found to contain 0.85 mg. of elemental chlorine per sq. cm. of fabric.

Chlorine may be removed from the fabric when it is desired to do so by rinsing the fabric in a solution containing a reducing agent. The fabric was rinsed in a 1 liter solution of water containing 2 grams of sodium thiosulphate and then dried. The fabric was analyzed and found to be free of elemental chlorine. Rechlorination can be effected as described above.

#### Example II

A monomethyloldicyandiamide and methylated trimethylolmelamine resin-treating solution is prepared by slowly adding with agitation 150 gms. of monomethyloldicyandiamide to a mixture of 98 gms. of phosphoric acid and 609 cc. of water (100° F.). The mixture is held below 120° F. and agitated until a clear solution is obtained. 366 gms. of methylated trimethylolmelamine is added to the solution and agitated until the solution again clears.

A 9 oz. cotton sateen fabric is padded with the resin-treating solution to about a 51% wet pick-up and dried at 200° F. The dried fabric is cured at 320° F. for 3 minutes. The resin-finished fabric is rinsed in clear water and dried. The fabric now has a permanent resin finish which will react with chlorine to form a vesicant protective finish. The fabric was immersed in a sodium hypochlorite solution containing 2.5% available chlorine for a 30-minute period and was rinsed in water, dried and exhibited excellent resistance to the passage of mustard vapors.

#### Example III

The impregnated fabric of Example II is alternatively cured by placing the padded fabric in an airtight container and held in this state for two hours at 210° F. to cure the resin. Thereafter, the fabric is dried, washed and dried. The resin finish is activated as in Example II and

the chlorinated resin finish exhibited increased stability of chlorine content over the dry, high temperature cure of Example II.

My invention would permit clothing to be permanently impregnated with the disclosed resins and, when exposure to vesicant agents is threatened, the clothing may be treated by immersion in a solution containing halogen ions, preferably positive chlorine ions. By impregnating military clothing with the disclosed resin finish, protection can quickly be obtained in the field by means of chemicals which are readily available thereby doing away with the necessity of stocking special purpose chemicals which can only be applied with difficulty or which cannot be securely attached to the fabric. Since my treatment permits after removal of the chlorine, garments can be hot-pressed without danger of fabric disintegration.

The invention described in detail in the foregoing specification is subject to changes and modifications without departing from the principle or spirit thereof. The terminology used is for purposes of description and not of limitation, the scope of the invention being defined by the claims.

I claim:

1. The method of providing an air-permeable protective fabric resistant to penetration of vesicant gases which comprises impregnating a fabric having at least a 50% fibrous cellulosic content with a methylol derivative of a nitrogenous resin-forming material capable of forming resins having sites which will react with chlorine ions to form N-chloramides, curing the resin-forming material on the fabric to form an insoluble resin finish permanently fixed to the fabric and wherein the amount of resin add-on is from 10% to 15% by weight of the dry fabric, and treating the resin-finished fabric with a chlorinating agent that will react with the resin and form the N-chloramides.
2. The method of claim 1 wherein the resin-forming materials are selected from the group consisting of methylol derivatives of urea, alkyl-substituted urea, melamine and dicyandiamide.
3. The method of claim 1 wherein the resin-forming material is monomethyloldicyandiamide.
4. The method of claim 1 wherein the cured resin is capable of combining with chlorine to effect a chlorine concentration of 0.1 to 1.0 mg. of elemental chlorine per sq. cm. of fabric.
5. A fabric produced by the method of claim 1.

#### References Cited

##### UNITED STATES PATENTS

|    |           |         |                     |          |
|----|-----------|---------|---------------------|----------|
| 50 | 2,628,174 | 2/1953  | Stokes et al. ----- | 117—62.1 |
|    | 2,659,681 | 11/1953 | Weldon -----        | 117—62.1 |
|    | 3,034,928 | 5/1962  | Prichard -----      | 117—143  |

55. MURRAY KATZ, *Primary Examiner*.

WILLIAM D. MARTIN, *Examiner*.

T. G. DAVIS, *Assistant Examiner*.